

## UNITED STATES PATENT OFFICE

2,041,120

HEAT AND SOUND INSULATING  
COMPOSITIONGeorge H. Ellis, St. Paul, Minn., assignor to The  
Insulite Company, Minneapolis, Minn., a corpora-  
tion of MinnesotaNo Drawing. Application March 1, 1934,  
Serial No. 713,517

4 Claims. (CL 106—18)

This invention relates to artificial sheet material fireproof in nature and adapted among other uses to employment as a structural unit. In various industries very large quantities of light sheet material are for use for insulating, as for example, in frame structures such as houses, refrigerators and the like. In addition to being light in weight such material should possess a marked degree of rot proofness and termite and fungi resistant qualities, be sufficiently stiff to hold its proper shape, should be effectively fireproof and to a certain degree sound absorptive. Due to these severe requirements the production of such material particularly in view of the fact that the great amount of material used necessitates the reduction of cost to the lowest possible point to admit a profitable sale thereof. Of course, reduction of cost may be obtained by use of cheap materials but such expedience ordinarily results in sacrificing in some degree one or more of the characteristics desired in an article of this kind.

The general purpose of the present invention is the provision of a fire-proof, sound-proof, rot-proof, and termite resisting structure which possesses the desired characteristics in adequate degree and yet may be produced at a relatively low cost.

Another object is the provision of a method for production of the article.

Other and further objects of the invention and the advantages of the same will be pointed out hereinafter indicated in the appended claims, or be obvious to one skilled in the art upon understanding the present disclosure.

For the purpose of this application there has been elected to set forth two particular structures and one particular method of producing the same, but it is to be understood that they are here presented for illustrative purposes only and are not to be accorded any interpretation such as might have the effect of limiting what is claimed as the invention short of its true and comprehensive scope in the art.

The article will be termed wood wool bat but it is to be understood that this term is not to be construed as a limitation upon the article produced.

Wood of a suitable character is divided into long slender pieces of what may be termed fine ex-

celsior. This material is then placed in a solution where it is saturated.

## Examples of satisfactory solutions

|                                      |       |       |    |
|--------------------------------------|-------|-------|----|
| I. Liquid                            | parts | 100   | 5  |
| Ammonium sulphate                    | do    | 8     |    |
| Ammonium phosphate                   | do    | 2     |    |
| Suitable toxic agent                 | grams | 60    |    |
| Hydrated wood pulp                   | parts | 10    |    |
| II. Liquid                           | parts | 100   | 10 |
| Ammonium sulphate                    | do    | 8     |    |
| Ammonium phosphate                   | do    | 2     |    |
| Dinitrophenol                        | grams | 30    |    |
| Wood pulp                            | parts | 10    | 15 |
| III. Liquid                          | parts | 50    |    |
| Silicate of soda                     | do    | 50    |    |
| Whiting                              | do    | 20    |    |
| IV. Water                            | parts | 300   | 20 |
| Zinc chloride                        | do    | 50    |    |
| Toxic agent                          | do    | 20    |    |
| Suitable pulp                        | do    | 20-30 |    |
| V. Liquid                            | parts | 100   | 25 |
| Termite and fungi resisting material | grams | 60    |    |
| Ground wood (or suitable pulp)       | parts | 8-15  |    |
| Water resisting material             | do    | 10-30 | 30 |

The wood wool should remain in the solution a sufficient length of time for the fireproofing solution and/or the water proofing material to penetrate the slender fibers. The time required for this depends upon a number of conditions, one being the temperature of the solution and another type and fineness of the wood wool. Very satisfactory results have been obtained by permitting wood wool to remain in the solution from 5 to 30 minutes.

A certain portion of the pulp used will adhere or cling to the wood wool and serves as a cementing material to bond the wood wool loosely together. After the wood wool has remained in the solution for a sufficient length of time for the material to penetrate the slender fibers the wood wool is removed and the free solution permitted to drain off. The wood wool is then formed into what would be termed a bat.

Any suitable batting equipment may be 50

utilized. For example a batting equipment may be used including a long screen apron having a vacuum box on the lower side thereof.

The wood wool is permitted to fall from a relatively great distance above the screen and the air passing through the screen distributes the wood wool uniformly over the surface of the screen and in a substantially heterogeneous arrangement.

Wood wool is deposited to a thickness depending upon the desired thickness of the finished product, for example, the wood wool may be deposited until it is approximately one foot in thickness and when thus deposited is very loosely arranged and highly porous.

15 The deposited material is then compressed to approximately 4 inches in thickness and is held under pressure while it is drying and the wood wool under these conditions has been found to have a very low conductivity and is suitable for 20 many uses. When applying pressure heat may be applied to expedite the drying and bonding.

It may be used for insulating frame buildings by filling the space between the studdings and the outside and inside of the walls. This arrangement of the insulating material prevents convection and transfer of heat from the inner wall to the outer wall and vice versa. One suitable way in which the material can be satisfactorily used in insulating frame buildings is by forming the 30 wood wool bat into bodies which are approximately  $14\frac{1}{2} \times 22\frac{1}{2}$  inches and of the desired thickness. As the finished bat is sponge like and easily compressible it will readily adjust its thickness and over all dimensions to compensate for 35 variations of space in the wall.

Of course it is to be understood that if the material is required to be water proof water proofing material of the proper kind is added to the solution in which the shredded material is 40 saturated.

This material also may be utilized in various ways and one of the modified ways of so using it is by depositing a relatively thin layer of the saturated fibers on the batting equipment and 45 securing by an adhesive, covering sheets. This will provide flexible sheets of material that may be used for linings. The adhesive used for securing the liners is preferably a fire-proof adhesive although it is not intended that the invention is to be limited to such an adhesive.

50 A preferable way of making a flexible sheet of the kind just described is to deposit the shredded

material on a support until approximately one to two inches in thickness and move this layer of material between covering sheets which have applied thereto an adhesive then subjecting the composite sheet to pressure while drying, and for 5 example is formed into sheets of approximately 10 feet in width and of any desired length. It may be applied by rolling the material against the studdings of the wall and then securing it to the studdings. The plaster receiving base may then 10 be secured to the studdings over the sheet of flexible material. This arrangement provides a wall of very low conductivity at a relatively low cost.

I claim:

1. A method of making fire resisting, sound 15 absorptive, insulating material which comprises reducing woody material to long, slender, curly shavings, preparing a fire resisting solution which includes two parts of ammonium phosphate and eight parts of ammonium sulphate, adding a 20 binder consisting of eight to fifteen parts of wood pulp, depositing the shavings in the solution for a time sufficient for the strands to become saturated, forming a relatively thick product from the shavings, and subjecting the product to 25 pressure while drying.

2. A method of making fire resistant, sound absorbent insulating material, which comprises reducing woody material to long, slender, curly shavings, depositing the shavings in a solution 30 including ammonium phosphate and ammonium sulphate, commingling a binder consisting of 8 to 15 parts of wood pulp, with the shavings forming a relatively thick product from the shavings, and drying the product. 35

3. A light, spongy, fire resisting bat, comprising a net work of slender, curly shavings of woody material saturated with a fire proofing solution which includes 2 parts of ammonium phosphate and 8 parts of ammonium sulphate, 40 and bound together by wood pulp, the pulp being present in an amount just sufficient to function as a binder.

4. A sound absorbing and fire-resisting bat, comprising a network of slender shavings of natural wood fire-proofed with materials which include ammonium phosphate and ammonium sulphate and bound together by wood pulp, the pulp being present in an amount just sufficient to 45 function as a binder. 50

GEORGE H. ELLIS.